

# United States Patent [19]

Pitton

[11] 3,920,488

[45] Nov. 18, 1975

[54] **PROCESS FOR COLORING ALUMINUM BLACK**

[75] Inventor: **Oscar Pitton, Schleitheim, Switzerland**

[73] Assignee: **Swiss Aluminium Ltd., Chippis, Switzerland**

[22] Filed: **Apr. 25, 1974**

[21] Appl. No.: **464,328**

[30] **Foreign Application Priority Data**

May 17, 1973 Switzerland ..... 7035/73

[52] **U.S. Cl. 148/6.27; 148/6.14 R; 148/6.2; 156/22; 427/287**

[51] **Int. Cl.<sup>2</sup> C23F 7/06**

[58] **Field of Search 148/6.27, 6.14 R; 156/22; 117/5.5; 204/38 A**

[56] **References Cited**

UNITED STATES PATENTS

2,285,468 6/1942 Slunder ..... 148/6.27

|           |        |                    |            |
|-----------|--------|--------------------|------------|
| 2,554,256 | 5/1951 | Lewis et al.....   | 148/6.27   |
| 3,326,728 | 6/1967 | Robinson .....     | 148/6.27   |
| 3,391,032 | 7/1972 | Hansen et al. .... | 148/6.27 X |
| 3,799,815 | 3/1974 | Subramaniam .....  | 148/6.27   |
| 3,833,374 | 9/1974 | Patrick.....       | 117/5.5    |

*Primary Examiner*—Ralph S. Kendall

*Assistant Examiner*—John D. Smith

*Attorney, Agent, or Firm*—Ernest F. Marmorek

[57]

## ABSTRACT

A process for producing, on aluminium and its alloys, matt black conversion coatings which bond well, are uniform and corrosion resistant. The metal surface is etched with an aqueous iron chloride solution, and then colored in an acidic, aqueous solution of ammonium molybdate and aluminium chloride and finally given an after-treatment with an aqueous, alkaline solution.

**11 Claims, No Drawings**

## PROCESS FOR COLORING ALUMINUM BLACK

The subject of the invention is a process for coloring aluminium and its alloys black.

Processes for coloring aluminium black are known, the coloring baths for which processes are based on ammonium molybdates and ammonium chloride. However the coatings obtained by these processes are covered with a dary grey powdery film, and the coating comes off easily when the aluminium is deformed.

The object of the invention presented here is to produce in a simple way on aluminium and its alloys, black conversion coatings which bond well to the substrate, are uniform and are corrosion resistant.

The object is fulfilled in terms of the invention in that the metal surface is etched in an iron chloride solution, then coloring in an acidic, aqueous solution of ammonium molybdate and aluminum chloride and finally is given an after-treatment with an alkaline aqueous solution.

With the process in accordance with the invention the following advantages are gained:

The presence of aluminium chloride in the coloring bath brings about a darker non-powdery coating which is not usually the case when the metallic parts are treated in a solution containing other chlorides.

- Surprisingly the properties of the film obtained can be significantly improved, in particular the corrosion resistance against alkalis.

Black conversion coatings produced in accordance with this process, are especially suitable for graphical reproduction processes:

An aluminium sheet which bears a conversion coating or an  $Al_2O_3$  coating after any desired process is covered with a photo lacquer. Those places, which should later be colored black, are covered with a negative. After exposure to light the lacquer can be removed easily from these places, whilst the other places which are covered with the polymerised lacquer after development and the oxide underneath are prevented from being colored black in the process. Thus the black areas, in contrast to those not attacked in the process, can be sharply delineated from areas which are white or which have another color. This is for example desirable with lettering, scanning or line-structured pictures.

Further features and advantages of the invention appear in the following description and examples.

The degreased articles which are made of aluminium or an aluminium alloy are first of all etched for 1 - 4 minutes in a 2 - 15 % aqueous iron chloride solution which is at a temperature of 70° - 95°C. The articles are then suspended for 0.5 - 10 min in a colouring bath at 80° - 92°C, containing 25° - 70 g/l, preferably 40 - 60 g/l ammonium-hepta-molybdate  $((NH_4)_6Mo_7O_{24} \cdot 4H_2O)$  and 10 - 100 g/l, preferably 40 - 80 g/l aluminium trichloride. The pH value of the bath lies between 2 and 5, preferably between 2 and 3 but must never fall below 2. At a bath temperature of 90°C the treatment time in the molybdate solution lies preferably between 2 and 8 min. Using a longer treatment time produces a thicker blue-black coating which does not bond.

In order to improve the corrosion-resistance the articles are finally given an after-treatment of 0.5 - 3 min

in an aqueous alkaline solution at 80° - 92°C. The treatment temperature is of greatest importance and lies between 85° and 92°C; at higher temperatures the coating becomes blue and does not bond so well, below 80°C the reaction is too sluggish.

The alkaline solution can contain either 10 - 20 g/l, preferably 13 - 17 g/l sodium chromate and 30 - 70 g/l, preferably 40 - 50 g/l sodium carbonate, or it can consist of a solution of ammonium or an ammonia derivative, for example hydrazine or hydroxylamine in a concentration of 10 - 20 g/l.

### EXAMPLE 1

Sheets of aluminium alloy containing 4.3 % Cu, 115 % Mg, 0.6% Mn, 0.4% Fe and 0.3% Si, and 100 × 70 × 1 mm in dimension, are after degreasing, suspended in a 5% iron chloride solution at 91°C for 3 minutes. After rinsing with cold tapwater the sheets are treated for 3 min in a solution of 5% ammonium hepta molybdate and 6% aluminium chloride at 91°C. The sheets obtain a grey-black coating.

After rinsing in cold tap-water the aluminium sheets are given a 1 min after-treatment with an aqueous solution of 1.5% sodium chromate and 5% sodium carbonate at a temperature of 90°C. The coatings obtained are smooth and black and exhibit a particularly good bonding base for the lacquer.

With one liter of coloring bath of the above mentioned composition, sheets of total surface area equal to 1.03 m<sup>2</sup> can be treated without being able to determine a change in colour tone and layer thickness. After 1.05 m<sup>2</sup> however the sheets are no longer black but begin to become increasingly gray and spotty.

### EXAMPLE 2

This example shows the influence of the after-treatment on the corrosion resistance. Aluminium sheets containing 1.1% Mn, 0.5% Fe, 0.3% Si and 0.1% Cu are divided into four parts A, B, C and D. Part A is treated as in example 1, whilst part B is given no after-treatment. Part C is treated only by the MBV process, and part D is anodised and colored black. The corrosion resistance of the treated samples A, B, C and D is tested in the salt spray test (3% NaCl at 35°C), the Kesternich test (artificial industrial atmosphere containing 0.66 vol % of both SO<sub>2</sub> and CO<sub>2</sub>) and the alkaline test (2% Na<sub>3</sub>PO<sub>4</sub>). The results are presented in tables 1 to 3.

Tables 1 and 2 show that sample A, with regard to corrosion resistance in the salt spray and Kesternich test, does not differ basically from sample C (classical alkaline chromatizing process) and D (anodised and then colored black in accordance with the usual process), although these are among the best known processes.

From table 3 it follows that anodised sheets (as for example D) have a low resistance to alkalis and, compared with sample A, suffer a large weight loss.

The process in accordance with the invention is therefore with respect to corrosion resistance at least the equal of other processes, but has the advantage over these, that it can be used without problem and without large expenditure for graphical reproduction purposes.

Table 1

## a) Salt-spray test

| Time (h) | Sample A                                                                    | Sample B                                                                                    | Sample C                         | Sample D  |
|----------|-----------------------------------------------------------------------------|---------------------------------------------------------------------------------------------|----------------------------------|-----------|
| 72       | unchanged                                                                   | attacked<br>2 pits/cm <sup>2</sup><br>~0.2 cm                                               | unchanged                        | unchanged |
| 144      | highly attacked<br>1-2 pits/cm <sup>2</sup><br>smaller than 0.2 mm          | strongly attacked<br>Change in colour tone,<br>5 pits/cm <sup>2</sup><br>from 0.5 to 0.8 mm | unchanged                        | unchanged |
| 216      | no change in colour<br>tone, 2-3 pits/cm <sup>2</sup><br>from 0.2 to 0.5 mm | destruction of the<br>coating                                                               | slight change in<br>colour tone  | unchanged |
| 480      | Change in colour tone,<br>4-6 pits/cm <sup>2</sup> ,<br>from 0.2 to 0.8 mm  | Blank aluminum,<br>no coating left<br>dark spots                                            | slight change in<br>colour tone, | unchanged |

Table 2

## b) Kesternich Test

| Time (h) | Sample A                                                                  | Sample B                                                                                                | Sample C                                    | Sample D                                                      |
|----------|---------------------------------------------------------------------------|---------------------------------------------------------------------------------------------------------|---------------------------------------------|---------------------------------------------------------------|
| 27       | Colour tone un-<br>changed, small<br>spots                                | more strongly at-<br>tached than sample<br>C, change in colour<br>tone                                  | Colour tone un-<br>changed, small<br>spots  | unchanged                                                     |
| 54       | strongly attached,<br>strongly attached,<br>large, white spots            | strongly attached,<br>marked change in<br>colour tone, but<br>very hard, dark grey<br>and rough surface | Change in colour<br>the layer flaked<br>off | tone, small<br>spots present                                  |
| 81       | strongly attached,<br>with large white<br>spots, change in<br>colour tone | Corrosion layer<br>thicker and harder                                                                   | destruction of the<br>coating               | marked change in<br>colour tone                               |
| 108      | as after 81 hours<br>but rather harder<br>layer                           | Grey corrosion<br>layer even thicker<br>and harder                                                      | no protective<br>layer left                 | no colour left<br>on the sheet,<br>oxide layer<br>became soft |

Table 3

c) Alkali resistance, 2 % Na<sub>3</sub>PO<sub>4</sub>

| Time<br>(h) | Anodised sheet,<br>Weight loss in<br>(mg/dm <sup>2</sup> ) | Aluminum<br>blank<br>(mg/dm <sup>2</sup> ) | Sample A<br>(mg/dm <sup>2</sup> ) | Sample B<br>(mg/dm <sup>2</sup> ) |
|-------------|------------------------------------------------------------|--------------------------------------------|-----------------------------------|-----------------------------------|
| 1           | 117                                                        | 26                                         | 6.5                               | 10                                |
| 2           | 229                                                        | 62                                         | 8.5                               | 12                                |
| 5           | 324                                                        | 89                                         | 23                                | 14                                |
| 10          | 380                                                        | 98                                         | 30                                | 26                                |
| 48          | 390                                                        | 114                                        | 36                                | 70                                |

## EXAMPLE 3

This example shows the influence of the time of treatment in the coloring bath on the growth of the layer, at constant temperature. The samples are treated as in example No. 1, the results are presented in tables 4, 5 and 6. In general almost all aluminium alloys can be colored black. The decisive parameter is the treatment time,

since the kinetics of the coating formation is dependent on the alloy composition.

## EXAMPLE 4

45 White anodised boards of 99.5 % purity aluminium are coated with a photosensitive lacquer using a known process, a negative is then laid on the lacquer and exposed to light. After the development only the non-exposed areas are etched until the white oxide skin is removed, the remaining areas are protected by the polymerised lacquer.

55 Boards treated this way are given a pre-treatment of 3 minutes in a 5 % iron chloride solution at 87°C, then suspended in a colouring bath in accordance with example No. 1 and finally given a very brief after treatment of 0.5 to 1 minute in a 2% aqueous hydrazine solution. Thus the previously non-exposed areas can be colored black, without a change in the anodic layer on the other areas being able to be observed.

Table 4

## Properties of the layers obtained in Example 3

| Aluminum<br>Alloy                 | Sample No | Treatment<br>time | Layer Weight<br>(mg/cm <sup>2</sup> ) | Colour                        | Remarks         |
|-----------------------------------|-----------|-------------------|---------------------------------------|-------------------------------|-----------------|
|                                   | 1         | 10 s              | 9,399                                 | iridescent to<br>yellow-brown | very thin layer |
| 1,5 % Mg<br>0,25 % Fe<br>0,2 % Si | 2         | 30 s              | 0,614                                 | yellow-brown                  |                 |

Table 4-continued

## Properties of the layers obtained in Example 3

| Aluminum Alloy | Sample No | Treatment time | Layer Weight (mg/cm <sup>2</sup> ) | Colour         | Remarks                                                                                    |
|----------------|-----------|----------------|------------------------------------|----------------|--------------------------------------------------------------------------------------------|
| 0.10% Mn       | 3         | 2 min          | 0.678                              | dark-brown     | well bonded layer, after treatment was black, in daylight after a few hours was dark brown |
|                | 4         | 3 min          | 0.734                              | brown to black | as with sample 3, after several hours of daylight was somewhat brown                       |
|                | 5         | 4 min          | 0.773                              | black          | no change of colour tone by daylight, bonded well                                          |
|                | 6         | 6 min          | 1.176                              | black          | as with sample 5, but slightly mottled                                                     |

After a treatment time of more than 6 min the layer thickness increases logarithmically, the bond strength becomes worse and the colour tone changes until it is dark blue. The optimum treatment time at constant temperature depends on the alloy used.

Table 5

## Properties of the layers obtained in Example 3

| Aluminum alloy                           | Sample No | Treatment time | Layer Weight (mg/cm <sup>2</sup> ) | Colour                            | Remarks                                                                     |
|------------------------------------------|-----------|----------------|------------------------------------|-----------------------------------|-----------------------------------------------------------------------------|
| 4.3% Cu<br>1.5% Mg<br>0.6% Mn<br>0.4% Fe | 1         | 3 s            | approx. 1.5                        | iridescent                        | bonded well                                                                 |
|                                          | 2         | 10 s           | 1.5                                | light brown with green reflection | bonded well                                                                 |
|                                          | 3         | 30 s           | 1.5                                | dark brown                        | bonded well and uniform                                                     |
|                                          | 4         | 2 min          | 1.8                                | dark brown to black               | bonded well and uniform                                                     |
|                                          | 5         | 3 min          | 2                                  | black                             | bonded well, treatment temperature not above 92°C, otherwise bluish coating |
|                                          | 6         | 4 min          | 2                                  | blue-black                        | layer did not bond as well as in the case of No 5                           |

With a treatment time of more than 4 min, the coating becomes dark blue and does not bond well.

Table 6

## Properties of coatings obtained in Example No 3

| Alloy                                    | Treatment time | Layer Weight (mg/cm <sup>2</sup> ) | Colour | Remarks                     |
|------------------------------------------|----------------|------------------------------------|--------|-----------------------------|
| 1.1% Mn<br>0.5% Fe<br>0.3% Si<br>0.1% Cu | 1              | 10 s                               | 0.285  | grey-yellow                 |
|                                          | 2              | 30 s                               | 0.25   | grey                        |
| 1.1% Mn<br>0.5% Fe<br>0.3% Si<br>0.1% Cu | 3              | 2 min                              | 0.399  | dark brown to black         |
|                                          | 4              | 3 min                              | 0.698  | black with brown reflection |
|                                          | 5              | 4 min                              | 0.763  | black                       |
|                                          | 6              | 6 min                              | 1.526  | black                       |
|                                          | 7              | 8 min                              | 1.527  | black                       |

If the treatment time is longer than 10 min then the layer exhibits white spots and no longer bonds so well. With no after-treatment a white powder forms on the black layer after a few days.

## What is claimed is:

1. A process for producing a matte black conversion coating on a metal surface of aluminum or its alloys which coating bonds well, is uniform and is corrosion resistant;

said process comprising the steps of:

etching said surface with an aqueous iron chloride solution; subsequently

coloring the etched surface in a coloring bath comprising an aqueous solution containing from about 25 grams to about 70 grams per liter ammonium-hepta-molybdate and from about 10 grams to

about 100 grams per liter aluminum trichloride; and thereafter

treating the colored surface in an after-treatment bath comprising an aqueous alkaline solution at a temperature of about 80°C to about 92°C.

2. A process as claimed in claim 1, wherein said coloring bath contains from about 40 to about 60 grams per liter ammonium-hepta-molybdate and from about 40 to about 80 grams per liter aluminum trichloride dissolved therein and has a pH value of 2 - 3.

3. A process as claimed in claim 1, wherein said after-treatment bath contains from about 10 to about 20

grams per liter sodium chromate and from about 30 to about 70 grams per liter sodium carbonate.

4. A process as claimed in claim 1, wherein said after-treatment bath contains from about 13 to about 17 grams per liter sodium chromate and from about 40 to about 50 grams per liter sodium carbonate.

5. A process as claimed in claim 1, wherein said after-treatment bath contains from about 10 to about 20 grams per liter ammonia or an ammonia derivative.

6. A process as claimed in claim 5, wherein said ammonia derivative is hydrazine or hydroxyl amine.

7. A process as claimed in claim 1, wherein the temperature of the after-treatment bath lies between 85° and 92°C.

8. A process as claimed in claim 1, said etching step further comprising using from about 2 to about 15 percent iron chloride at a temperature of about 70°C to about 95°C and etching the surface therewith for about one to about four minutes.

9. A process as claimed in claim 1, wherein said coloring bath has a pH value from about 2 to about 5 and a temperature from about 80°C to about 92°C further comprising the step of coloring said surface from about 0.5 to about 10 minutes.

10. A process as claimed in claim 1, further comprising the step of using said conversion coatings for graphical reproduction processes.

11. A process for producing a matte black conversion coating on a metal surface composed of aluminum or its alloys, which coating bonds well, is uniform and is corrosion resistant;

said process comprising the steps of:

etching said surface with an aqueous solution containing from about 2 to about 15 percent iron chloride for about one to about four minutes at a temperature of about 70°C to about 90°C; subsequently

coloring the etched surface from about 0.5 to about 10 minutes in a coloring bath comprising an aqueous solution having a pH value of about 2 to about 5 and containing from about 25 grams to about 70 grams per liter ammonium-hepta-molybdate and from about 10 grams to about 100 grams per liter aluminum trichloride, said coloring bath being at a temperature of approximately 80°C to approximately 92°C; and thereafter

treating the colored surface in an after-treatment bath for about 0.5 to about 3 minutes, said after-treatment bath comprising an aqueous alkaline solution at a temperature of about 80°C to about 92°C.

\* \* \* \* \*

30

35

40

45

50

55

60

65